

May 7, 1940.

L. A. KLEBER

2,200,178

## PRODUCTION OF COMPOSITE CASTINGS

Filed March 8, 1938

Fig. 1.



Fig. 2.



*Luther A. Kleber* Inventor

By *Jack Richardson*

Attorney

## UNITED STATES PATENT OFFICE

2,200,178

## PRODUCTION OF COMPOSITE CASTINGS

Luther A. Kleber, High Bridge, N. J., assignor to  
 Taylor-Wharton Iron & Steel Company, High  
 Bridge, N. J., a corporation of New Jersey

Application March 8, 1938, Serial No. 194,654

15 Claims. (Cl. 22—201)

The invention provides certain improvements in composite castings and in the methods thereof and more particularly it provides for the production of tubular or hollow cylindrical shapes, comprising cylindrical sections, formed, respectively, of different metals joined end to end, in such way as to insure homogeneous union of the sections and in such way as to inhibit substantial penetration of the metal of one section into the metal 10 of the other section, meaning by that such interpenetration as may have the effect of so altering the characteristics of the section encroached upon as to render it unfit to perform the particular service for which it was intended.

15 It is more or less common knowledge that if a molten metal of a certain analysis be poured onto a molten metal of a different analysis each will intimately mix with the other to form one mass, the analysis of which will be some combination of the two original analyses. There is no particular problem in such casting operation and for some classes of work the castings are satisfactory. On the other hand, there are certain kinds of service employing composite cast cylindrical shapes for which it is desirable, if not essential, to have definite lengths of different analyses. For example, the casting may be required to withstand high heat at one end and to conduct heat rapidly at the other end as when employed 25 as an inner barrel in heat accumulator stoves of the Aga type. Excluding certain comparatively rare and high cost metals, the metals capable of withstanding high heat are otherwise not satisfactory because of their low rate of heat conductivity.

30 Recourse has been had to the riveting and otherwise mechanical connection of separate castings and they even have been welded together but there are many objections to such practice aside from the fact that they are not economical.

40 It has been proposed to produce composite cast stove elements, such as inner barrels and the like, by separately pouring, into one and the same mold, pig iron forming one cylindrical section and ferrochrome forming the other cylindrical section, reliance being had upon a chill to, in effect, dam the ferrochrome and prevent it from rising through the pig iron. This practice suffers the objection of lack of control of the 45 height and character of the line of merger between the two metals because the first metal is poured to a point below the level of the chill so that the second metal encounters the chill before any welding can take place with the first metal 50 and, consequently, there is ever present the hazard,

ard of a poor weld especially since no provision is made for getting rid of impurities carried to the welding area by one or both metals.

It is the purpose of the invention to obviate the difficulties and disadvantages of the conventional practice and, briefly stated, it provides a method and means whereby in the composite casting of inner barrels and the like some of one or the other or of both metals is permitted to flow off at or adjacent their point of mergence for the purpose and with the result of flushing away any impurities that may be present and which, if allowed to remain, would militate against sound welding, said flowoff having as its main purpose and result the positive control of the composite casting operation by serving to establish the level of the weld within closely reckoned limits, that is to say, within about an inch (1/2" plus or minus of the theoretical).

It is characteristic of the invention that it will insure the production of sound castings regardless of the presence or absence of chills, whether internally or externally applied, and regardless of the compositions of the metals to be joined. And yet, it is a merit of the invention that it admits of the use of inserts or chills which I have devised in the nature of coils or helices of light strand wire which, while effective in the performance of their chilling office, offer no serious obstacle to metal flow but permit the metal to flow freely through the coils and about the strands so that for all practical purposes the wire is fused and a cross section of the casting in the chilled area will show substantially solid metal. So also it is a merit of the invention that unusually good results follow the use of the metal composition hereinafter stated.

The invention in its preferred embodiment will be described in connection with the accompanying drawing in which

Figure 1 is a sectional view of the improved mold.

Figure 2 is a section on line 2—2 of Fig. 1, showing the general construction and arrangement of one of the coil chills.

The mold 5 is equipped with separate pouring provisions 6 and 7 for bottom and top pouring. The practice heretofore has been first to pour the ferrochrome through the pouring provision or gate 6 and then to pour the pig metal or cast iron via the gate 7 and, while the order and metals may be reversed according to the problem in hand, I adhere to that practice except that, in any event, I provide at a predetermined point in the common mold cavity a metal flowoff 8. For

example, assuming the presence of a chill insert 9 in the bottom poured metal 10 the flowoff is located above the chill but with or without chills, and regardless of the order of casting, the flowoff 5 8 is arranged so that it will be effective to run off some of one or both metals to flush away impurities and to insure sound metal in the region of the consolidation or mergence of the two metals while controlling interpenetration. Sufficient 10 amounts of both metals may be poured to insure a proper run off at 8, but it is manifestly more economical to rely principally on excess pouring of the baser metal as the flushing medium.

While the flow-off 8 is the dominating factor in 15 controlling interpenetration of the separately cast metals, that is to say, fusion of the metals and a clean weld of sound metal within closely reckoned limits, for example within about an inch (1/2" plus or minus of the theoretical) there are 20 occasions in the quantity production of shapes when it is desirable to employ chills and the flow-off 8 admirably lends itself to coordination in that practice regardless of the form and arrangement of the chill or chills and whether they 25 be inserts or applied in any other conventional way. However, when an insert is deemed expedient or desirable I find it good practice to employ one and preferably two coil chills arranged one above the other and so disposed that the 30 metal first poured will be above the upper chill. Such chills are illustrated as rings 9 of helical or coiled iron wire. In the production of inner barrels, and the like cylindrical castings, I find that wire of about .050 gage in the form of coils 35 whose outside diameter is about 5/8th" to be adequate for the purpose. Coiled wire chills are advantageous because they offer no serious check to metal flow to the desired level and yet accelerate the cooling rate so that there can be no 40 excessive or undesirable interpenetration of the metals.

When applying my invention to the production of solid cast heat accumulator units, such as inner barrels, I prefer to employ metals of analyses 45 substantially as follows, more or less,

Cast iron:

|    |            |              |
|----|------------|--------------|
| 50 | Carbon     | 3.00 to 3.50 |
|    | Silicon    | 1.75 to 2.50 |
|    | Manganese  | .40 to .60   |
|    | Sulphur    | .10 to .12   |
|    | Phosphorus | .40 to .50   |

Chrome cast iron:

|    |            |                |
|----|------------|----------------|
| 55 | Carbon     | 2.00 to 2.50   |
|    | Silicon    | 1.30 max.      |
|    | Manganese  | .60 max.       |
|    | Phosphorus | .26 to .35     |
|    | Chrome     | 28.00 to 32.00 |
|    | Molybdenum | .50 to .60     |

The molten chrome cast iron is preferably 60 poured first through the gate 6 whence it passes to the bottom of the mold and rises through the chills 9 to the level indicated by the line X which is substantially the top level of the flow-off 8. The cast iron is then poured via the sow gate or 65 pouring basin 7, and some of it is permitted to flow away at 8 to displace some of the first poured metal, to obviate the presence of impurities, to insure sound metal in the zone of fusion and to control the depth of interpenetration substantially 70 within predetermined limits. After sufficient lapse of time to satisfy the requirements of such flushing and control the flow-off 8 is plugged as at 11 and the pouring of the cast iron is continued until the remainder of the mold cavity and the riser, 12 are filled.

During the casting the coils 9 serve to accelerate the cooling rate of the metal surrounding them and as some of this metal is essentially above the coil or chill, the chrome cast iron is prevented from undesirably penetrating the cast 5 iron and vice versa. The penetration is indicated at 13 and it is restricted to definite limits, as previously stated, the depth of penetration being a line in the plane of the upper level of the flow-off and, at any rate, above the chill. 10

While not essential to the practice of the invention, the presence of a chill 14 in the top of the heavy cast iron section operates to improve the appearance of the eventually machined surface 15 through a reduction of graphite precipitation in the cast iron metal and by causing the graphite to precipitate in fine particles rather than in the form of coarse flakes. 15

In service, as stove heat accumulator units, long periods of high temperatures are alternately applied to the chrome cast iron section with no ill effects such as distortion, cracking or growth. The cast iron is sufficiently removed from high temperature concentration to avoid the faults of growth and distortion common to this metal 25 when exposed to high temperatures for long periods. Heat is rapidly conducted through it and the temperatures are high enough to suit the purpose completely. The two metals, in the solid cast association described, are ideally suited to all 30 service requirements.

This application is a continuation of application Serial No. 69,578.

What is claimed as new:

1. Method of making castings having defined 35 areas differing in analytical, physical and structural attributes, which consists in pouring into a mold cavity a metal of predetermined analysis, and before it solidifies pouring in endwise relation a metal of different analysis, and preventing substantial interpenetration of the two metals by chilling one or the other poured metal at a point immediately adjacent the zone of fusion.

2. Method of making heat accumulator units for stoves of the sealed type, which consists in 45 forming as an integral casting a shape having defined areas of different attributes by successively pouring metals of different analyses and controlling the mergence of the metals by applying chills at a point immediately adjacent the zone of 50 fusion to define the areas.

3. A stove heat accumulator unit comprising cast bound sections whereof one is constituted of cast iron and whereof the other is constituted of chrome cast iron, the metal of one of said 55 sections being poured around a chill insert arranged closely adjacent the line of fusion whereby the mergence of the metals is substantially confined to the zone of fusion.

4. Method of making solid cast heat accumula- 60 tor units comprising chrome cast iron and cast iron in which said respective metals are limited to definite endwise sections of the casting, which comprises casting the sections separately in endwise arrangement while introducing a chill at 65 the zone of fusion to limit penetration of the metal of one section into the metal of the other section.

5. Method of making solid cast heat accumula- 70 tor units comprising cylinders of chrome cast iron and cast iron, respectively, having a substantially clearly defined line of demarcation, which consists in casting the shapes in the order stated under fusing conditions, and preventing the cast iron from substantially penetrating the

- chrome cast iron by accelerating the rate of cooling of the chrome cast iron in the immediate area of the zone of fusion.
6. Method of making solid cast heat accumulator units comprising cast bound cylinders of chrome cast iron and cast iron, respectively, having a substantially clearly defined line of demarcation, which consists in casting the shapes in the order stated under fusion conditions, and preventing the cast iron from substantially penetrating the chrome cast iron by introducing a ring chill into the chrome cast iron at its point of mergence with the cast iron.
7. Method of making solid cast heat accumulator units comprising cast bound cylinders of chrome cast iron and cast iron, respectively, having a substantially clearly defined line of demarcation, which consists in casting the shapes in the order stated under fusion conditions, and preventing the cast iron from substantially penetrating the chrome cast iron by introducing a ring chill into the chrome cast iron at its point of mergence with the cast iron, and chilling the remote end of the cast iron to reduce the amount of graphite precipitation.
8. A heat accumulator unit comprising cylindrical shapes of chrome cast iron and cast iron, respectively, in cast bound arrangement, the chrome cast iron shape having a chill insert to inhibit substantial penetration by the cast iron, and the cast iron section having a chilled area at its outer end to cause a reduction of graphite precipitation.
9. The method set forth in claim 1 in which some of the molten metal is run off in the vicinity of the chilling area so as to remove impurities and to insure homogeneous union of the separate metals.
10. Method set forth in claim 1 in which the chilling is effected by an annular chill constructed as an open coil and interposed in the path of the bottom poured metal at or about the level of the flowoff.
11. An inner barrel comprising cast bound aligned tubular sections whereof one is constituted of cast iron and whereof the other is constituted of chrome cast iron, the chrome cast iron being poured through and around a ring chill comprising an open coil, said chill being arranged closely adjacent the line of fusion whereby the mergence of the metals is substantially confined to the zone of fusion and yet the metals are homogeneously united due to the substantial presence of cast metal throughout the chill.
12. Method of making solid cast heat accumulator units comprising barrel shape units welded together in end to end relation and formed, respectively, of chrome cast iron and cast iron, which comprises substantially simultaneously casting the barrel sections in endwise arrangement, the first metal being poured through and beyond the level of an open helical chill to limit penetration of the metal into the second poured metal, and adjusting said level to insure sound welding metal by flowing off some of one or both metals at or about the zone of fusion. 10
13. Method of making solid cast heat accumulator units comprising end to end cast bound hollow cylinders of chrome cast iron and cast iron, respectively, having a substantially clearly defined line of demarcation, which consists in casting the shapes in end to end relation under fusion conditions and with provision for mutual washing of the eventual welding areas, and preventing the chrome cast iron from substantially penetrating the cast iron by introducing a ring chill in the form of an open coil into the chrome cast iron at an effective point below its mergence with the cast iron. 15
14. A heat accumulator unit comprising a barrel formed of half barrels joined end to end and composed, respectively, of chrome cast iron and cast iron, the chrome cast iron shape having a ring chill insert comprising a ring coil to inhibit substantial penetration by the cast iron, and the cast iron shape having a chilled area near its outer end to reduce the amount of graphite precipitation. 30
15. In the composite casting of structures which in service are exposed to high temperatures and so prone to separate, said structures comprising barrel shape members arranged end to end and composed, respectively, of chrome cast iron and cast iron, the steps which comprise 35 pouring the metals separately towards a common point of mergence, limiting interpenetration of the metals in order to maintain their separate identities by chilling the metals at or about the zone of fusing by causing the cast iron without appreciable interruption of its flow to traverse an open helical chill, and flowing off some of the cast iron at or about the zone of fusion so as to insure homogeneous union of the separate metals. 40

LUTHER A. KLEBER.